

## UNITED STATES PATENT OFFICE.

ROBERT HOPFELT, OF HAMBURG, GERMANY, ASSIGNOR TO THE FIRM METALLISATOR  
BERLIN AKTIEN-GESELLSCHAFT, OF BERLIN-NEUKOLLIN, GERMANY.

METHOD FOR PREVENTING SCORIFICATION OF FIRE BARS, GRATE SURFACES, AND  
THE LIKE.

No Drawing. Application filed January 29, 1925, Serial No. 5,661, and in Germany partly on February 28, 1924.

It is known to prevent scorification of, or formation of slag on, grate-surfaces, fire- or furnace-bars and the like, while at the same time increasing the fire proof quality of the metal, by providing it with a layer of aluminium on such places as are subjected to the action of heat and the influence of slag. This layer is produced by projecting divided aluminium in a molten state against the surface to be coated, and thereupon slowly heating the work piece to a temperature approximating the melting temperature of the metal of the work piece. The idea was that by the subsequent heating of the work piece thus besprinkled with aluminium an alloying between the aluminium and the ground metal takes place. This, however, is an erroneous conclusion. The aluminium which has been applied to the work piece in a cold state is very porous, and since aluminium easily oxidizes, this porous aluminium layer in the subsequent treatment eagerly takes up oxygen and is thus turned into aluminic oxide which for itself adheres only loosely to the thus coated article. When such a coated and heated work piece is cooled down the coating generally scales off quickly, the more so when the work piece is subjected to mechanical treatment while in the fire, particularly by pokers, rakes or stoke bars.

It has been moreover proposed to produce an alloying of the metal coating with the ground metal by subsequently heating the besprinkled work piece in an inert gaseous atmosphere, consisting for instance of nitrogen or hydrogen. Even such method fails with aluminium not to speak of the fact that it is extremely costly and complicated and requires exceptionally precautions measures.

The substance of the present invention is a method which allows fire bars or the like to be provided with an aluminium coating in such manner that it adheres extraordinarily firmly by intimately alloying with the ground metal, and besides makes the surface of the work piece so hard that it withstands all thermic and mechanical treatment much better than all heretofore known fire-bars, no matter how the composition is effected.

The invention is based on the discovery that aluminium adheres with absolute certainty, for instance to an iron work piece, when the latter is heated previously to a temperature in which the aluminium melts.

The preheating of a work piece to be besprinkled is in itself known. However, for the present object this measure of preheating the work piece is not sufficient. Care must be taken, that, when it is desired to attain the object of the present invention, the surface of the work piece while being preheated does not oxidize, because only with such precautions does a flowing together of the aluminium projected on the heated work piece, with the ground metal of the work piece, takes place. Theoretically such oxidation could be prevented even, it is true, in such way as is known by allowing the preheating of the work piece to take place in an indifferent gaseous atmosphere. Practically, however, it is either impossible to have recourse to this way or only possible with extraordinary difficulties, because aside from the difficulties spoken of above in connection with the use of an indifferent gaseous atmosphere it would be necessary to take care that the projecting of the aluminium should also take place within this atmosphere, and even before the work piece comes in contact with air whereby it would be oxidized.

The invention follows therefore a quite different course; according to which a thin aluminium layer is projected on the work piece in a cold state, which layer should be just so thick that the surface of the work piece is protected against oxidation. The work piece thus provisionally coated is heated up to about 800° C. that is to say to a temperature which is approximately the melting point of the aluminium. When on such heating the provisional layer of aluminium is turned partly into aluminic oxide this will not be of any harm, because this aluminic oxide layer fulfills its purpose to protect the ground metal against oxidation, it not being acted upon mechanically.

When now in this heated state of the work piece another aluminium layer is projected upon the previously applied coating to the required thickness, this aluminium layer combines intimately with the ground metal because the provisionally projected porous and thin aluminium layer will be penetrated by the particles of the finally projected aluminium layer which casts aside any oxides that might have been created by the provisional aluminium layer, and such oxides would be made harmless by being encased or reduced.

When thus the final aluminium layer is applied by projection to the sufficient thickness, now the known subsequent treatment can take place by again heating or again raising the temperature of the besprinkled work piece to 1000° C. and more. Since then an intimate reciprocal contact of the ground metal and the projected aluminium has taken place an even alloying of the two metals 10 over the complete area results, and in this manner alloys of almost any composition between the ground metal and the aluminium can be carried out, by appropriate choice of the amount of the projected aluminium 15 and of the temperatures in the subsequent treatment.

Under certain circumstances the subsequent heating may be omitted, that is to say when the work piece during the ordinary 20 treatment has been subjected to sufficient heating, which when it is carried out sufficiently long, need not arrive at 1000° C.

When the work pieces treated according to the new method described above are examined by the microscope, it will be found 25 that the aluminium layer has been intimately combined with the ground metal over the complete surface to form an alloy if the ground metal is steel or wrought iron. 30 However, the adhering is not so complete on certain places of the surface of the work piece if this consists of cast iron. Therefore it can be concluded that cast iron work pieces have spots or places in which free carbon is present to a greater amount, which 35 prevents the formation of alloy, and therefore an unevenness in the adhering of the coating results.

Starting from this discovery according to 40 a further feature of the invention the work pieces, as far as they contain larger amounts of carbon, will be superficially freed from such carbon in an atmosphere, which is preferably not oxidizable, and which comprises 45 constituents which with carbon are turned into a gaseous combination or which consists of such. In the first instance for such atmosphere hydrogen is well adapted, particularly in the form of illuminating or burning 50 gas, which combines with carbon to form

hydrocarbon. Also nitrogen is applicable since it forms cyanogen gas or ammonia. It is sufficient if the surface only is decarbonized, since only this is to alloy with the coating. The annealing of the work piece 55 can take place either in a state when not yet besprinkled or eventually then when the first thin aluminium layer has been applied. In the latter case the annealing must be very 60 exactly regulated and care must be taken, to increase the temperature only slowly, so as not to prevent a timely harmless escape of the gaseous carbon combinations through the pores of the coating by an untimely condensing of the still porous coating, and thus 65 the creation of blisters and scaling off of the second final coating is prevented. The annealing, after the first coating has been applied, has the advantage that it can be combined with the heating of the article up 70 to the melting temperature of aluminium, which in any case is necessary as the first operation.

It may be still further remarked that the superficial decarbonizing of work pieces, 75 which are to be tinned or zinned by the aid of bodies which give off oxygen in the heat, is known. From this known method the present differs according to the invention inasmuch as the annealing for the purpose of 80 superficial decarbonization takes place in a non-oxidizing atmosphere.

I claim:

A method for preventing the scorification 85 of fire or furnace bars, grates and the like comprising projecting molten aluminium against the cold work-piece to form upon it a preliminary firmly adherent coating, heating the coated workpiece to approximately 90 the fusion temperature of the aluminium, thereby alloying the inner portion of said coating with the workpiece, the outer portion becoming oxidized and projecting a subsequent quantity of molten aluminium 95 against said coated workpiece while still in its heated state, thereby breaking through the layer of oxide and forming an integral accretion to the inner alloyed portion, producing a coating of any desired thickness.

ROBERT J. HOPFELT.